

## UNITED STATES PATENT OFFICE

ROBERT A. MARR, OF NORFOLK, VIRGINIA, ASSIGNOR TO RAMAR SYNDICATE INCORPORATED, OF NORFOLK, VIRGINIA, A CORPORATION OF VIRGINIA

## CEMENTITIOUS PRODUCT AND PROCESS OF OBTAINING SAME

No Drawing. Application filed January 12, 1924, Serial No. 685,895. Renewed July 31, 1926.

The present invention relates to a new product, namely, intercellular cementitious matter of wood, or other plant growth which can be obtained as a by-product, or used in combination with the fibrous content, in the manufacture of pulp and paper and fibrous material, from wood, including both hard and soft woods, also including cane or bamboo, banana stalks, and to some extent the invention 5 embraces somewhat similar products made from marsh grasses, sedges and similar growths.

In my U. S. Patent No. 1,166,848 I have described the manufacture of pulp and paper, 15 by a process involving the digestion of wood and various other materials, with zinc sulfate solution, which may also contain other chemicals.

In my Patent No. 1,362,723 I have described the production of textile fibers by a similar digestive treatment. In a copending application, Serial No. 407,759 filed September 2, 1920, I have described the use of solutions of sulfate of iron, sulfate of copper, and various 25 other sulfates, as digestive fluids, in which to treat wood or other materials for the production of paper and pulp and fibrous materials. In my copending application 595,215 filed October 17, 1922, I have described the digesting of cane, either alone or mixed with various other woods, in digestive fluids containing zinc sulfate, potassium sulfate, or sodium sulfate, or mixtures of these sulfates, with or without others. In my application 30 616,609 filed February 2, 1923, I have described the use of aluminum sulfate or magnesium sulfate, sodium sulfate, potassium sulfate, or mixtures of the same, for digesting wood or cane material or mixtures of such 35 materials. In my copending application 616,610 I have described the use of solution of kainit (a complex material saline deposit containing potassium sulfate, magnesium sulfate and magnesium chloride) as a component of the digestive fluid.

In all of the above cases, the sulfates themselves form the active chemical constituents of the digestive fluid, and it is not necessary to use sodium sulfide, caustic soda or the like, 40 for the digestion of such materials as above

stated. In all of the above cases the time for cooking can be an hour or a few hours, and it is not necessary to employ a long period such as 8 or 10 hours up to 30 or 40 hours at high pressure, as in some of the prior processes proposed for the production of paper pulp, according to the prior art. The strength of the digestion solution as employed in my above mentioned cases, varies more or less, but in all cases is preferably substantially 55 less than 5% and in many cases even as low as 1 or 2% solution has been found to give very satisfactory results. The digestion can be carried out in the ordinary digestors, made say of cast iron, as commonly 60 used in the art.

In all of the above cases, the materials treated may be any of the ordinary woods, or cane, bamboo or various other vegetable materials, or mixtures of such materials, and the named materials all contain a substantial amount of intercellular cementing material, by which the fibers or fiber bundles are bound together in the original vegetable growth. After the digestion has been completed, the 70 material can be run between rolls, or run through a pulper with water, or otherwise crushed and thereby reduced to a pulp, containing about 100% of the content of the material used, excepting water solubles. The 75 pulp can be used like pulp produced by other methods, for the production of paper or the like.

I will state that a particular digestive solution which has been found to give very satisfactory results, is one made by mixing two parts of zinc sulfate, one part of potassium sulfate, and two parts of sodium sulfate, and dissolving each in water and making the digesting solution, in the proportion of say, 80 1.5 to 3 ounces of total salts per gallon, and another very satisfactory solution is one produced by mixing two parts of magnesium sulfate, two parts of sodium sulfate and one part of potassium sulfate, dissolving this 85 mixture in water, in the proportion of about 1.5 to 4 ounces per gallon. These two solutions have been found to give very satisfactory results with all kinds of woody materials, straw, marsh growth, cane, bamboo, banana 90 95

stalks and similar materials. While under some conditions, any of these sulfates can be used alone, it is found that when the fibrous or woody material under treatment contains a large percentage of silica in any form (e. g. bamboo, canes, etc.) it is advisable to use potassium sulfate as one of the ingredients of the digestive solution, in order to prevent the formation of gelatinous silica compounds.

10 As in my cases as above referred to, the digestive solution can be used over a considerable number of times and it is not necessary to evaporate the liquid to dryness and to calcine the materials each time, as has been the usual practice with the chemicals used 15 in some of the other processes heretofore proposed.

10 In carrying out the digestive process, apparently a small part of the carbohydrate constituents of the cementitious matter of the wood are converted into something resembling sugars, and these sugars are somewhat caramelized, during the cooking process, which gives a more or less brownish color 25 to the pulp, and also gives a characteristic caramel-like odor to the digestive fluid after the same has been used one or more times.

10 After the digestive operation, the wood or other material can be pulped in any suitable manner, with water, in order to mechanically shatter the intercellular cementitious binder to some extent, although the same does not become soluble in my process, as in the processes heretofore generally used for pulp 35 manufacture. After the pulping operation above referred to, the material can be washed or can be run directly into a beating engine, and can be beaten therein, in accordance with the usual practice for a desired length of 40 time, to convert the same into a pulp. It is preferable in most cases to operate the beater with the roll raised a considerable distance above the bed, particularly at the commencement of the beating operation. The 45 roll can be gradually brought down during the beating operation, towards the bed-plate, and if desired, the beating operation can be continued for say, one to two hours, during which time the roll will be brought 50 down to say 1 to 2 turns above the bed, in order to give a brush beating effect without cutting or shortening the individual fibers.

10 The cementitious materials, including the air duct and xylose systems, as is shown by 55 microscopic investigation, and by actual practice, are largely reduced to extreme fineness, but to not become soluble. For this reason, by my processes, the pulp or paper stock runs freely on the Fourdrinier wire cloth, without 60 clogging the latter and all resinous matters seem to be agglutinated to the fiber without clogging the wire mesh.

10 During or after the beating operation (or 65 after the pulping operation whether or not the pulp is to be beaten) a considerable pro-

portion of the cementitious matter in the pulp can be removed, which operation can be conducted in an ordinary pulp washer, or the beater may carry a co-ordinated washer for removing any desired part of the cementitious matter, during the beating operation, thus leaving when desired, clean, clear, individual fibers, free from the finely divided inter-cellular cementitious material.

10 Some kinds of pulps, that is to say the pulps from some of the above mentioned woody materials, are found to be improved somewhat for some purposes, by removing a portion of the cementitious matter in the mode above described, and the amount to be removed will depend upon the particular kind of pulp under operation, and the particular properties of the desired final pulp product. The fraction of the cementitious matter removed may be 5% to 12% based on the total 15 quantity of the wood or other material. This removal can be made by means of a screen forming a part of the pulp washer, or other separating device. In some cases the pulp as coming from the pulper, without going to a beater, can be washed to separate therefrom any desired portion of the intercellular cementitious material, and the washed pulp can be turned into wet or dry laps which reduce 20 in a short time equally as well, to liquid pulp. Hence cheap semi-portable plants can operate 25 where the said material is found and the plants moved to new sources of supply; the wet or dry pulp being shipped to permanent paper products mills.

100 There is in all cases produced a slurry containing cementitious matter of wood, in a considerable amount of aqueous liquid, such as water, and the slurry can be allowed to settle whereby the cementitious matter drops 105 out of the liquid vehicle, the latter can be decanted off, or the liquid can be drained off, say by the use of fine sieves, or equivalent arrangement. If desired, a filter press, or centrifugal separator, can be used, through 110 which the entire amount of liquid from the pulp washing operations can be passed and the filter cake will consist of the cementitious matter of plant growth usually with a small 115 proportion of the finer fibers.

120 The cementitious matter can be run into molds, when carrying any desired percentage of water, say as a mass of the consistency of mortar or putty which does not stick to the fingers. This can be pressed into the desired shape, and the molded articles can be dried in the molding press or after being taken out of the press. If desired, fillers 125 can be incorporated with the cementitious matter, before or at the time of molding. Water-proofing agents can be added to the paste of the cementitious matter, before molding or the molded articles can be treated with a waterproofing agent. Suitable water-proofing agents are rosin size, rubber latex,

oil emulsions, asphalt emulsions or mixtures of these, and suitable precipitants can be incorporated therewith, either before molding or after molding or after molding and drying. The molded articles can also be subjected to a vulcanizing treatment, whether or not waterproofing agents (such as latex, rosin etc.) have been used. I find that addition of a small proportion of latex to the rosin size before adding the latter, aids in the agglutination of the intercellular cementitious material (e. g. one part latex to 2-3 parts rosin size) followed by a precipitant, say alum.

The molded articles (when no fillers or other admixtures are used) are light in weight and normally of a brownish color (in the air-dry state) about the color of hemlock-tanned leather, but can be made of any desired color, by the use of dyes, etc. They are also (even if no water-proofing agent is used) quite water-resistant, after air-drying, so that they can be soaked in water, for days and months at a time, without becoming wet through. In fact a small piece (after drying in the air) immersed in water for about 24 hours was found, on examination, to be covered with a thin film of water, but the water had not penetrated the surface at all, so far as could be observed; the examination being made after breaking the piece.

When it is desired to further waterproof the articles, the pasty mass of the cementitious binder can be mixed with, say, 2 to 10% of rubber latex, before the molding operation. The molded articles, with or without waterproofing agents, when molded under pressure are strong, light and rigid, and rather tough, and take a good polish.

In certain of the appended claims, I employ the term "wood" and I intend thereby to designate products which are distinctively lignified, such as hard woods, soft woods, cane, bamboo, and banana stalks, as distinguished from such materials as grasses, sedges and the like, which are of herbaceous nature.

I claim:

1. A process which comprises digestively cooking cellulosic material in a solution containing a sulfate, such solution being of a concentration substantially below 5%, thereafter pulping the cellulosic material and separating a substantial part at least of the disintegrated cementitious connective matter from the pulp, and thereafter isolating such separated cementitious connective matter, and molding the same.

2. Disintegrated cementitious matter of vegetable growth, separate from the fibrous matter of such vegetable growth, and in an undissolved water-insoluble condition.

3. A process which comprises digesting wood in a solution containing a sulfate, such solution being of substantially less than 5% strength, and the digesting operation continued until the cementitious matter in the wood

is rendered friable, but not until the major proportion of the same is dissolved, thereafter liberating at least a considerable portion of the cementitious matter in an undissolved condition into a bulk of aqueous liquid, and recovering a part at least of the said cementitious matter from said liquid.

4. Disintegrated cementitious matter of vegetable growth, separate from the fibrous matter of such vegetable growth, and in an undissolved water-insoluble condition, such material being molded into form, and substantially waterproof.

5. A material including the disintegrated but undissolved cementitious matter of wood, substantially free from the cellulosic fibers.

6. A product including the disintegrated but undissolved cementitious matter of vegetable growth, which material is capable of being molded, either alone or in combination with other materials but free from large amounts of the long cellulose fibres of the original vegetable growth.

7. The herein described disintegrated but undissolved cementitious matter of wood, or mixtures containing the same, which material is capable of being formed and worked and water-proofed, and which material itself upon drying is capable of hardening to a solid state, such product being substantially free from cellulose fibers.

In testimony whereof I affix my signature.  
ROBERT A. MARR.

70

75

80

85

90

95

100

105

110

115

120

125

130